

## UNITED STATES PATENT OFFICE

2,216,605

## ELECTROPLATING

Samuel Sklarew, Yonkers, and Lionel Cinamon,  
New York, N. Y., assignors to Special Chemicals  
Corp., New York, N. Y., a corporation of New  
York

No Drawing. Application March 30, 1938,  
Serial No. 198,826

2 Claims. (Cl. 204—44)

Our invention relates generally to electroplating and more particularly, to a novel electroplating bath.

One of the objects of our invention is to provide a novel electroplating bath of the character described which is adapted to electrodeposit a novel and highly improved alloy plate.

Another object of our invention is to provide a novel electroplating bath of the character described which is adapted to electrodeposit a novel and highly improved alloy plate upon zinc die cast objects and which is at the same time highly resistant to corrosion.

A further object of our invention is to provide an electroplating bath which will deposit a copper-cobalt-tin alloy plate of the character described with consistently satisfactory results and in a simple and inexpensive manner.

Other objects of our invention will in part be obvious and in part hereinafter pointed out.

In accordance with our invention, a dry composition, that is, an electroplating bath composition, may be prepared by making a mixture of copper salts, cobalt salts, tin salts and an alkaline cyanide. This composition is added to water or any other suitable solvent to form an electroplating bath solution from which may be electrodeposited upon an object, in a manner and by means well known in the art, an alloy plate comprising copper, cobalt and tin.

We have found that when an electroplating bath solution, prepared in accordance with our invention, contains a copper content of from about 0.04 to 15.85 grams per gallon, a cobalt content of from about 0.02 to 9.2 grams per gallon, and a tin content of from about 0.02 to 3.6 grams per gallon, a satisfactory copper-cobalt-tin alloy plate may be electrodeposited therefrom. It is understood, however, that our invention is not to be construed as being limited by these ranges.

In supplying the copper, cobalt and tin contents of the bath, any salt or salts of copper, cobalt and tin may be employed in the dry plating composition which, when combined with other ingredients comprising the plating composition, will dissolve in the solvent employed. Some of these salts are:

50 Sodium stannate  $Na_2SnO_3 \cdot 3H_2O$   
Stannous phosphate  $Sn_3(PO_4)_2$   
Stannous tartrate  $SnC_4H_4O_6$   
Copper cyanide  $Cu_2(CN)_2$   
Copper sulphate  $CuSO_4$   
Copper tartrate  $CuC_4H_4O_6$   
55 Cobaltous sulfate  $CoSO_4 \cdot 7H_2O$

Cobalt tartrate  $CoC_4H_4O_6$   
Cobalt carbonate  $CoCO_3$   
Cobalt cyanide  $Co(CN)_2 \cdot 2H_2O$   
Sodium cobaltocyanide  $Na_4Co(CN)_6$   
Cobalt phosphate  $Co_3(PO_4)_2$

5 Sufficient alkaline cyanide should be mixed into the dry bath composition to ensure a free or uncombined alkaline cyanide content in the electroplating bath of from 0.3 ounce to 6 ounces per gallon. We have found that the 10 most satisfactory results are obtained by the presence of 2 to 3 ounces of free alkaline cyanide per gallon.

In connection with the practice of our invention, suitable plating voltages, temperatures and 15 current densities generally known to the art may be employed.

By our invention, salts of copper, cobalt and tin may be satisfactorily used to electrodeposit a bright plate from an alkaline cyanide electro- 20 plating bath for periods of time up to one minute, without the necessity of employing any addition salts for brightening or conductivity. The electroplate thus obtained suffices for an inexpensive and practical plate on articles such as 25 those used in the novelty trade.

When a heavier and more durable plate is desired, we have found that addition agents as 30 brighteners and for conductivity, such as those listed below, may be used.

Tri-sodium phosphate  $Na_3PO_4 \cdot H_2O$   
Rochelle salt  $NaKC_4H_4O_6 \cdot 4H_2O$   
Potassium thiocyanate  $KCNS$   
Sodium bisulfite  $NaHSO_3$   
Sodium sulfate  $Na_2SO_4$   
Sodium carbonate  $Na_2CO_3$   
Sodium arsenite  $NaAsO_2$   
Di-sodium phosphate  $Na_2HPO_4$   
Sodium pyrophosphate  $Na_4P_2O_7 \cdot 10H_2O$   
Arsenious acid  $As_2O_3$   
Sodium phenylate (phenate)  $NaC_6H_5O$   
"Goulac" (tailings from sulphite liquor concentrate in preparation of wood pulp)  
Sodium thiosulfate  $Na_2S_2O_3$   
Soda alum  $Na \cdot Al(SO_4)_2 \cdot 12H_2O$   
45 Glucose  $C_6H_{12}O_6$   
Dextrose  $C_6H_{12}O_6$   
Dextrine  $(C_6H_{10}O_5)_x$   
Ammonium molybdate  $(NH_4)_6Mo_7O_24 \cdot 4H_2O$   
Sodium oxalate  $Na_2C_2O_4$   
Ammonium hydroxide  $NH_4OH$   
Bone glue  
Thiourea  $NH_2-CS-NH_2$   
Potassium ferrocyanide  $K_4Fe(CN)_6$   
The above-listed addition salts are represen- 55

tative members of their groups. For example, Rochelle salt is a member of the tartrate group and merely given as an example of such. Other tartrates, such as ammonium, copper, magnesium, cobalt or tin tartrate, would cause the plating bath to function equally well.

We have found that satisfactory results are obtained by using the following addition salts for brightening or conductivity either singly, 10 doubly, or in multiple combination in the ranges set forth.

| 15 | Addition agents      | Satisfactory ranges       | Preferred amounts    |
|----|----------------------|---------------------------|----------------------|
|    |                      | Grams per gallon          | Grams per gallon     |
|    | Tri-Sodium phosphate | 0.01 to 100               | 28.3                 |
|    | Sodium arsenite      | 0.01 to 1                 | 0.1                  |
|    | Di-sodium phosphate  | 0.01 to 1                 | 0.1                  |
|    | Rochelle salt        | 0.01 to 1                 | 1.0                  |
| 20 | Arsenious acid       | 0.01 to 1                 | 0.01                 |
|    | Sodium phenylate     | 0.01 to 1                 | 0.01                 |
|    | Sodium pyrophosphate | 0.01 to 1                 | 0.01                 |
|    | "Goulac"             | 0.01 to 1                 | 0.1                  |
|    | Sodium bisulfite     | 0.01 to 1                 | 0.1                  |
|    | Sodium sulfate       | 0.01 to 1                 | 0.05                 |
|    | Sodium thiosulfate   | 0.01 to 1                 | 0.1                  |
| 25 | Soda alum            | 0.01 to 1                 | 0.05                 |
|    | Glucose              | 0.01 to 1                 | 1.0                  |
|    | Dextrose             | 0.01 to 1                 | 0.1                  |
|    | Dextrine             | 0.01 to 1                 | 0.05                 |
|    | Bone glue            | 0.01 to 1                 | 1.0                  |
|    | Ammonium molybdate   | 0.01 to 1                 | 0.3                  |
|    | Sodium oxalate       | 0.01 to 30                | 14.15                |
| 30 | Ammonium hydroxide   | Cr. per gallon<br>5 to 30 | Cr. per gallon<br>15 |

We have found that the double combinations of addition agents listed below also give good results:

(Grams per gallon)

|    |                           |       |                      |
|----|---------------------------|-------|----------------------|
| 40 | 0.01 Di-sodium phosphate  | +1.0  | Rochelle salt        |
|    | 0.01 Sodium pyrophosphate | +0.01 | Sodium phenylate     |
|    | 0.1 "Goulac"              | +0.01 | Tri-sodium phosphate |
| 45 | 0.1 Sodium bisulfite      | +1.0  | Rochelle salt        |
|    | 0.05 Sodium sulfate       | +0.1  | "Goulac"             |
|    | 0.1 Sodium triosulfate    | +1.0  | Rochelle salt        |
|    | 0.1 Sodium thiosulfate    | +0.01 | Sodium phenylate     |
| 50 | 0.1 Sodium thiosulfate    | +0.1  | Sodium bisulfite     |
|    | 0.05 Soda alum            | +1.0  | Rochelle salt        |
|    | 1.0 Glucose               | +0.01 | Arsenious acid       |
|    | 1.0 Glucose               | +0.01 | Tri-sodium phosphate |
| 55 | 0.1 Dextrose              | +0.01 | Sodium phenylate     |
|    | 0.1 Dextrose              | +0.1  | "Goulac"             |
|    | 0.05 Dextrine             | +0.01 | Sodium phenylate     |
|    | 1.0 Bone glue             | +0.01 | Sodium bisulfite     |
|    | 1.0 Bone glue             | +0.05 | Sodium sulfate       |
|    | 1.0 Bone glue             | +0.05 | Soda alum            |
| 60 | 1.0 Bone glue             | +1.0  | Glucose              |

The following are specific examples of dry bath compositions which we have found to give good results, it being understood that they are in no way limitative. The weights given are for use with one gallon of a plating bath.

#### Example I

|    | Grams            |        |
|----|------------------|--------|
| 70 | Sodium stannate  | 8.60   |
|    | Sodium cyanide   | 90.00  |
|    | Copper cyanide   | 18.00  |
|    | Cobalt carbonate | 5.80   |
|    |                  | 122.40 |

#### Example II

|                  |        |
|------------------|--------|
| Sodium stannate  | 8.60   |
| Sodium cyanide   | 90.00  |
| Copper cyanide   | 18.00  |
| Cobalt carbonate | 5.80   |
| Rochelle salt    | 1.25   |
|                  | 123.65 |

#### Example III

| Grams                |        |
|----------------------|--------|
| Sodium stannate      |        |
| Sodium cyanide       |        |
| Copper cyanide       |        |
| Cobalt carbonate     |        |
| Rochelle salt        |        |
| Tri-sodium phosphate |        |
|                      | 131.25 |

#### Example IV

| Grams                |        |
|----------------------|--------|
| Rochelle salt        |        |
| Sodium stannate      |        |
| Tri-sodium phosphate |        |
| Sodium cyanide       |        |
| Copper cyanide       |        |
| Cobaltous sulfate    |        |
|                      | 139.25 |

We have found that by our invention a ferrocyanide, such as potassium ferrocyanide, may be used to partially replace sodium cyanide in the bath and reduce the effect of carbonate formation from the breakdown of sodium cyanide as is illustrated by the following example:

| Grams           |       |
|-----------------|-------|
| Cobalt cyanide  |       |
| Sodium cyanide  |       |
| Copper cyanide  |       |
| Sodium stannate |       |
|                 | 82.00 |

Potassium ferrocyanide 1 to 10 grams.

By our invention, as above described, we have been able to produce an electroplated alloy, characterized by its whiteness which approaches silver, has a high reflectivity, and is at the same time hard and ductile so that metals upon which our alloy has been electrodeposited may be formed without peeling, chipping or cracking. Also, our alloy plate forms a substantially uniform deposit on irregular surfaces due to the high throwing power of the solution. Also, it is highly tarnish-resistant, being unaffected by salt spray, mustard and olives, lemon juice, or the like. The alloy plate is moreover resistant to corrosion by cold caustic or alkaline solutions of any strength and can only be slowly dissolved by any single acid, so that it furnishes a good foundation or primary plate because other plates, such as a chromium plate or a nickel plate, may be readily stripped therefrom without affecting it. This latter characteristic of the alloy plate produced by our invention, namely its excellence as a primary plate, is particularly important in regard to zinc die cast objects on which primary electroplates have heretofore tended to be absorbed or become blistered, or on which difficulty has been experienced in electrodepositing a second plate. We have found that our novel bath will electrodeposit a smooth plate on zinc die cast objects which will not be absorbed and may be used as a base plate for other electrodeposits having any specially desired characteristics.

It will thus be seen that there is provided a

composition, bath and process by means of which the several objects of this invention are achieved, and which are well adapted to meet the conditions of practical use.

5 As various possible embodiments might be made of the above invention, and as various changes might be made in the embodiments above set forth, it is to be understood that all matter herein set forth is to be interpreted as illustrative and  
10 not in a limiting sense.

Having thus described our invention, we claim as new and desire to secure by Letters Patent:

1. A process of electrodepositing a white copper-cobalt-tin alloy plate comprising passing current through an aqueous alkali cyanide bath  
15 solution containing copper salts, cobalt salts and tin salts, the quantities of said salts being

such that the metallic contents of one gallon of said solution will be from about 0.04 to 15.85 grams of copper, from about 0.02 to 9.2 grams of cobalt, and from about 0.02 to 3.6 grams of tin, and having a free alkali cyanide content of from 5 0.3 to 6 ounces per gallon of solution.

2. An electroplating bath for depositing a white alloy plate of copper, cobalt and tin, said bath comprising an aqueous alkali cyanide solution of copper, cobalt and tin salts and from 0.3 to 6 10 ounces of free alkali cyanide per gallon of solution, said bath having metallic contents per gallon of solution of from about 0.04 to 15.85 grams of copper, from about 0.02 to 9.2 grams of cobalt and from about 0.02 to 3.6 grams of tin. 15

LIONEL CINAMON.  
SAMUEL SKLAREW.